

June 30, 1931.

C. W. BENNETT

1,812,508

METHOD OF MAKING SHEETS AND PLATES

Filed June 21, 1927

3 Sheets-Sheet 1



*Fig. 2.*



Witness

*Edwin Trueb*

by:

*Inventor:*  
CHARLES W. BENNETT,  
D Anthony Usina  
his Attorney.

June 30, 1931.

C. W. BENNETT

1,812,508

## METHOD OF MAKING SHEETS AND PLATES

Filed June 21, 1927

3 Sheets-Sheet 2



*Witness*

Edwin Trub

*Inventor:*  
CHARLES W. BENNETT,  
By:

D. Anthony Usina  
his Attorney.

June 30, 1931.

C. W. BENNETT

1,812,508

METHOD OF MAKING SHEETS AND PLATES

Filed June 21, 1927

3 Sheets-Sheet 3



Fig. 9A.



Fig. 9B.



Inventor:  
CHARLES W. BENNETT,

D. Anthony Neira  
his Attorney.

Witnesses

Edwin Trumbull

## UNITED STATES PATENT OFFICE

CHARLES W. BENNETT, OF PITTSBURGH, PENNSYLVANIA, ASSIGNOR TO AMERICAN SHEET AND TIN PLATE COMPANY, OF PITTSBURGH, PENNSYLVANIA, A CORPORATION OF NEW JERSEY

## METHOD OF MAKING SHEETS AND PLATES

Application filed June 21, 1927. Serial No. 200,423.

The invention relates to the manufacture of rolled metal sheets and plates, and more particularly to the manufacture of light gage black plates of the class used in making tin plate.

5 One object of my invention is to provide a novel method of rolling sheets and plates in which reduction of the metal in the rolling operations is effected in a new and improved manner, and by which sheets and plates are produced, wherein variations in the gage of different sheets and plates and also in different parts of single sheets or plates are reduced to a minimum, when not entirely 10 avoided and overcome.

15 In making sheets and black plates by existing methods it is the general practice to roll these materials from sheet bars, such bars approximating eight inches in width. The 20 bars vary in length and also vary in gage and, because of differences in length and gage, in weight. The length of the sheet bars is governed by the width of the sheets or black plates to be made, and the thickness or gage 25 and weight of the bars is determined by the length and gage of the sheets or plates into which the bars are rolled.

30 The sheet bars when being rolled extend lengthwise parallel with the axis of the rolls. At the commencement of the rolling operation, single bars are rolled on a two-high roughing mill. In this operation two bars are rolled at the same time, although they are 35 passed singly between the rolls, one bar being handed over the top roll of the mill by the "catcher" while the other is being passed between the rolls by the "roller". The single bars, after being given several passes, usually five, are matched by laying one on top of 40 the other to form a pair and the matched pair is then given a few passes, usually three, in the roughing mill, so as to further elongate the metal and lessen its gage. The matched pair is then doubled, to form a pack 45 of four thicknesses of metal, and again heated. The reheated pack is then again rolled on a two-high finishing mill, usually being given three passes, after which it is again doubled into a pack of eight thicknesses. 50 The pack of eight is then sheared on the

open end and reheated, after which it is given two or three passes in the finishing mill, which finishes the sheets in the pack to the specified finished length.

The above described operations which are typical of the methods in general use, are varied to suit conditions, packs of three being formed in some cases and, when making very light gages, packs of six, twelve, or more thicknesses of metal being rolled in the finishing mill.

Hot finished sheets and plates and particularly the light gages of black plates used in making tin plate, must have smoothly finished surfaces and be as nearly uniform and accurate in gage as is possible, because in many cases the use to which the tin plate may be put depends upon its surface condition and exactness to gage.

My invention provides an improved method in which accuracy of the gage of the finished sheets and plates is influenced and to a large extent controlled from the commencement of and throughout the series of rolling operations. By starting with a slab of calculated weight, which is afterward rolled into a thin flexible strip of relatively great length and by cutting the thin strip into sections in the novel way forming part of this invention, the production of materials of improved 70 finish and desired accuracy of gage is made possible. 75

In making sheets and black plates by methods embodying my invention, the ordinary, universally used sheet bars are not used, a 80 slab large enough to make a series of packs of sheets or black plates being employed instead of the sheet bars. As each slab forms a plurality of packs, and each pack a known 85 number of sheets or plates, the slab necessarily will be of much greater size and weight than the usual pair of sheet bars ordinarily used in forming a pack for rolling such sheets and plates. 90

Referring now to the drawings forming part of this specification—

Figure 1 is a perspective plan showing an ingot after being rolled to the width and thickness of the slabs into which the rolled 100

ingot or manifold length slab is afterward sheared.

Figure 2 is a perspective plan showing diagrammatically a single slab and the number 5 of ordinary sheet bars of which it is an equivalent in size and weight.

Figure 3 is a perspective plan showing the long, thin, flexible strip into which the single slabs of Figure 2 are rolled in practicing my 10 invention (the thickness of the strip relative to its width and length, as shown, being exaggerated), and also showing the way in which the long, thin strip is cut into strip sections of uniform weight in accordance with my invention.

Figure 4 is a perspective plan showing a pair of the strip sections into which long strips like that of Figure 3 are cut and matched preparatory to being doubled.

20 Figure 5 is a perspective plan showing the matched pair of strip sections of Figure 4 as doubled, to form a pack of "fours," preparatory to rolling the so-formed pack to length and gage in a finishing mill.

25 Figure 6 is a perspective plan illustrating the pack of "fours" of Figure 5 after being partly rolled, preparatory to being doubled into a pack of "eights."

30 Figure 7 is a perspective plan showing the rolled pack of "fours" of Figure 6 as it is doubled to form a pack of "eights" preparatory to reheating and rolling in a finishing mill, to gage and length, when rolling packs of "eights" is contemplated.

35 Figure 8 is a perspective plan illustrating the pack of "eights" of Figure 7 after being rolled to elongate and reduce it in thickness and form sheets or plates of the desired gage.

40 Figures 9A and 9B, when joined on the lines IX-IX, form a diagrammatic plan showing a preferred form of mill adapted for use in carrying out my improved method.

45 Figure 10 is a diagrammatic side elevation showing a pile of the long, thin strips, the spacing shear by which the single strips are cut from the multiple length strips, and the doubler by which matched pairs of the single strips are doubled into packs of "fours."

50 In the accompanying drawings, the numeral 2 designates the heating furnace in which the slabs are heated in preparation for rolling them. These furnaces, of which three are shown, preferably will be continuous furnaces of the gravity discharge type shown, wherein the slabs are charged into the furnace at or near one end and are discharged at or near the opposite end, through a suitable opening at the end or else in the furnace bottom.

60 Located in line with each other and with the slab discharge openings of the heating furnaces 2 is a series of stands of reducing rolls forming a continuous mill by which the short, thick slabs A of Figure 2 are rolled into the long, thin strips E of Figure 3.

The first stand of rolls 3 is a two-high stand of horizontal edging rolls to which the individual slabs A are delivered edgewise from the furnaces 2. On the discharge side of the rolls 3 is a slab shear 4 by which double length slabs are cut into single slabs, as is necessary in some cases. (For example, when the single slabs A are so short that delivery of them from the furnaces 2 would be difficult.)

75 On the discharge side of the shear 4 are two-high stands of rolls 5<sup>a</sup> and 5<sup>b</sup> forming the first and second of the flat reducing passes in the continuous mill. On the discharge side of the rolls 5<sup>b</sup> is a universal mill consisting of a pair of vertical rolls 6<sup>a</sup> and a pair of horizontal rolls 6<sup>b</sup>, the vertical rolls 6<sup>a</sup> rolling the edges of the metal delivered from the rolls 5<sup>b</sup>. A single stand of vertical edging rolls may be substituted for the universal mill 80 formed by the pairs of rolls 6<sup>a</sup> and 6<sup>b</sup>, when found desirable.

85 As shown, a two-high stand of rolls 7<sup>a</sup> and six four-high stands 7<sup>b</sup>, 7<sup>c</sup>, 7<sup>d</sup>, 7<sup>e</sup>, 7<sup>f</sup>, and 7<sup>g</sup> are located on the discharge side of the universal rolls 6<sup>a</sup>, 6<sup>b</sup>, these rolls forming a series of successive flat passes by which the metal is further elongated and reduced in gage. The top and bottom rolls of the four-high stands are backing-up rolls which enable 90 greater reductions in thickness of the metal in the successive passes. The number of stands of rolls used to form the continuous mill, and the number of four-high stands 95 shown are merely illustrative and obviously may be varied as is found necessary or desirable.

100 Suitable feed tables (not shown) will extend between the furnaces 2 and the edging rolls 3. Also between the rolls 3 and slab shear 4, and from the shear 4 to the rolls 5<sup>a</sup>, and similar feed tables will be provided between the succeeding stands of rolls 7<sup>a</sup>, 7<sup>b</sup>, 7<sup>c</sup>, 7<sup>d</sup>, 7<sup>e</sup>, 7<sup>f</sup>, and 7<sup>g</sup> to convey the metal from one stand to the next and away from the last 110 roll stand 7<sup>g</sup>.

115 At the end of the continuous mill are tracks 8 for the trucks or cars on which the strips, while still heated from the rolling operations, as delivered from the continuous mill and while still heated from the rolling operation, are formed into piles, and a turn-table 9 at the ends of the tracks 8, and having tracks 10, is employed to turn the loaded trucks at right-angles to the tracks 8 and deliver them onto the tracks 11.

120 An overhead traveling crane (not shown) removes the piles of rolled strips and delivers them to the storage beds 12 at the rear of the spacing shears 13. In front of each spacing shear 13, of which there are four shown, is a matcher and doubler 14 by which a plurality of successively sheared strip sections are matched and doubled, in the practice of my invention.

The doubled packs K are then stored until required for rolling into sheets or plates. When used, the doubled packs are taken to hot mills of the usual construction whereby they are heated, and the heated packs are then rolled on the hot mills to length and gage in the usual known manner.

In practicing my improved method, an ingot of suitable size and weight will be rolled into a long slab of known width and thickness or gage. The manifold length slab will then be cut into single slabs A or, in some cases, into slabs of double length. Each slab A (as is shown in Figure 2) will have a width B substantially the same as that of the sheets or plates to be rolled from the slabs. The slabs have an arbitrarily fixed thickness C and a length D, which, after making due allowances for loss by oxidation in heating and in rolling, as well as for the scrap or discard formed in shearing the finished sheets or plates to length and width, will have the amount or weight of metal required to form the predetermined number of packs of sheets, when rolled into a strip E.

Stated another way, the slab length D will equal the weight per foot of eight inch sheet bars required for a given order of sheet bars, multiplied by a factor, this factor taking into account the number of packs of eight sheets each that is to be made from the slab, plus the loss of metal in the slab heating and rolling operations and in the scrap formed in shearing off or cropping the ends of the strip.

For example, assuming that fourteen packs of eight sheets each are to be made from each slab A in filling an order, and that in the continuous mill there is a scrap loss of 5.625 per cent., the factor 2.9 times the sheet bar weight (in pounds per foot) used on this order under the old method of rolling will give the slab length D in inches. For the average run of gages and pack lengths rolled, the slab lengths will range between 25 and 42 inches.

The factor 2.9 is typical of the rolling practice from slab to finished sheet or plate for a given mill but it should be understood that a factor may be readily computed for any mill where the scrap loss in the continuous mill varies from the figure of 5.625 or where the hot mill practice under the old method of rolling has dictated a different range of sheet bar foot weights for specified gages of sheets or plates.

Each slab A, after first being heated, is rolled, preferably in a continuous mill like that shown in the Figure 9A of the drawings and is thereby formed into a long thin and flexible strip E having a width F which is substantially the same as the slab width, a thickness G approximating .05 inches (18 gage) and a length H of from 80 to 170 feet.

It being impracticable to heat all of the

slabs equally or uniformly, the temperature at which any one slab is rolled will vary from that of others when rolling the slabs into strips of a size and weight for filling a given order. The result of such unequal rolling 70 temperatures is that, although rolled close to the desired gage or thickness, the gage of each multiple length strip E will vary somewhat from that of others of the same lot of strips. It is obvious that the thicker strips 75 will be of less length than the thin ones.

Because of these practical conditions it follows and will be readily seen that if the successively rolled strips E should be cut to a constant length, some of the strip sections I, 80 would be heavier than others and that this difference in the weight of the strip sections I would be reflected in the pack length of packs of the sheets or plates later rolled from different strips. This might result in such an 85 excessive scrap loss and such variations in the gage of the sheets or plates in the successively rolled packs as to become prohibitive.

The difficulties are readily overcome in practicing my improved method because of 90 the novel way in which the multiple length strip E is cut into strip sections I, as will now be described.

In forming the strip sections I, a spacing shear 13, preferably an automatic spacing shear, is employed, this shear enabling a multiple length strip to be cut into a predetermined number of sections of equal length or of lengths which vary by pairs in regularly increasing or decreasing proportion. 100

The spacing shear 13 employed in shearing the long strips into sections is preferably of the single cut type, although shears of the type using a plurality of sets of cutting knives may be used if desired. The long strip is run into shearing position with the front end of the strip projecting beyond the shear knives just sufficiently to cut off the scrap end. At the same time a marker or target on the shear (not shown) is set up at 105 the rear end of the strip at the point where, when the strip is sheared, the rear scrap end or fishtail will be cut off. This marker or target is connected to the shear feeding mechanism in such manner that when the shear is placed in operation the strip will be fed forward and sheared into a predetermined number of sections of equal length or into sections of different lengths, the lengths varying by pairs in regularly increasing or decreasing proportion. 115

The result is that each length strip E is cut into the same predetermined number of pieces or strip sections I and although the length of the strip sections may vary, they all will have a constant or substantially constant weight or, what is the same thing, each strip section although differing somewhat in gage or in length from the others, will have the right amount of metal to make with a second 120

strip section a doubled pack of the required size.

- 5 The strip sections are then matched in pairs J and the pairs are then doubled by the doubler 14 to form a pack K of four thicknesses of one-half the length of the matched sections. In finishing them, the doubled packs K are first reheated and are then rolled in a two-high finishing mill, into a rolled 10 pack L of the desired length and gage, or else to a degree of thinness that makes further heating desirable or necessary, as is the case when the material is to be finished in packs of eight thicknesses of metal.

- 15 When to be further rolled, the now elongated pack L of four thicknesses, before it is reheated, is again doubled and in this way formed into a pack of eight thicknesses of metal. After being thus doubled, the pack 20 M is reheated and again rolled in the finishing mill until it has been elongated to the required length, which also reduces the pack M to a finished pack N of eight thicknesses of the desired gage. The rolled packs N are 25 then sheared to dimensions and, after being sheared, are separated and finished in the usual known manner. In fact, the matching, doubling, and rolling operations after the strip sections are cut may be, and preferably 30 are, the same as are carried out in existing methods of rolling sheets and plates from sheet bars after the sheet bars are roughed down and first doubled.

- 35 The long thin strips E rolled from the slabs A on the continuous mill ordinarily will emerge from the last stand of rolls 7<sup>g</sup> at a temperature high enough to make it desirable to pile the strips quickly so as to minimize oxidation and to contribute the flatness 40 and in this way facilitating subsequent operations when reducing to thin sheets or plates. In performing this piling operation the long strips E are pushed sidewise off the run-out table onto buggies or trucks on the tracks 8, 45 the piles being built up on alternate sides of the run-out table. The piles, which, as completed, are from 12" to 18" in height, are moved to the spacing shears 13 where the strips E are fed singly to one or another of the shears 13 and are cut into the predetermined 50 number of sections as has been described.

- 55 A plurality of the strips may be fed to the shears instead of singly, when found desirable or necessary. When the strips E are found to be sufficiently uniform in length to permit feeding a plurality of them to the spacing shears, the shearing operating is facilitated and the necessity of matching a plurality of the cut sections I is avoided.

While it is not new to use mechanical doublers in making hot rolled sheets and tin plates whereby packs of heated sheets or plates are doubled at different stages of the rolling operations, I believe it is new to em-

ploy doublers in the location and in the manner described herein, as in practicing my improved method, the doublers form part of the spacing shear units and are used in connection therewith. The long strips E as sheared at the spacing shears 13 when sheared singly are immediately matched one on top of the other in two or more thicknesses and passed to the table of a doubler 14 and when sheared in multiple thicknesses, not requiring matching, they are passed directly to the doubling table, and in either case being doubled into packs of four, six or more thicknesses.

The doubled packs, when made in this manner, are then placed on crates or racks in orderly piles for removal in lots of several tons at a time to the furnaces for reheating preparatory to hot rolling. The furnaces, which preferably will be continuous furnaces, will be so arranged that the crates of doubled packs are set at the rear of the furnaces and the doubled packs are fed forward, one at a time, from the crates or piles into and through the furnaces to emerge at the opposite ends in position to be fed to the hot mills for further reduction.

The advantages of my invention, which will be apparent to those skilled in the art, result from the novel form of slab used in making the strip sections from which the plates are rolled and the way in which strip sections of uniform width and substantially uniform gage and weight are formed.

While certain specific steps of the method in certain relation to each other have been described, it is to be understood that the invention is not limited thereto, since various modifications may be made without departing from the invention as defined in the appended claims. Slabs made in accordance with my invention may also be employed in rolling single sheets or in rolling packs of two, three, five or six thicknesses of metal.

The length of the strip sections cut from a multiple length blank may vary progressively from one end to the other of the long thin strip to compensate for differences in gage at different points in the length of the multiple length blank, provided the predetermined number of multiples fixed upon in calculating the weight of the slab is preserved.

For example, eight pieces or strip sections may be cut from a strip of forty feet in length, or sixteen sections from one of eighty feet, or thirty-two pieces from a strip of one-hundred and sixty feet in length. In such cases the first two sections cut from the multiple length strip may be somewhat longer or shorter than the last two, with a graduated difference for each pair of the intermediate strip sections, this being done to take care of the differences in gage from end to end that may, and usually do, occur in hot rolled strips.

of such length. The exact amount of variation in length that is necessary will readily be determined by gaging a long strip at different points in its length and proportioning the length of the predetermined number of cuts in pairs from shorter to longer, corresponding to the gage variation. The spacing shear will do this for a known gage variation from end to end of the strip.

I claim—

1. The method of making sheets and plates, which consists in cutting long metal slabs of known width and thickness into slabs of the length and weight necessary to make a predetermined number of packs of sheets or plates, rolling the cut slabs into long thin flexible strips of known width and gage, and then cutting each rolled strip into a predetermined number of duplicate sections, matching a plurality of the strip sections and rolling the matched sections into sheets or plates of the desired length and gage and determining from the overall length of the long, flexible strip the length into which the individual sections are cut.

2. The method of making sheets and plates, which consists in cutting long metal slabs of known width and thickness into slabs of the length and weight necessary to make a predetermined number of packs of sheets or plates, and rolling the cut slabs into long thin flexible strips of known width and gage and then cutting each rolled strip into a predetermined number of duplicate sections, and varying the length of the sections into which individual strips are cut to compensate for variations in the temperature at which a series of strips are successively rolled and thereby form strip sections of accurate and uniform weight, matching a plurality of the strip sections and rolling the matched sections into sheets or plates of the desired length and gage.

3. The method of making sheets and plates, which consists in cutting long metal slabs of known width and thickness into slabs of the length and weight necessary to make a predetermined number of packs of sheets or plates, and rolling the cut slabs into long thin flexible strips of known width and gage, then cutting the rolled strips into a predetermined number of sections and thereby form duplicate strip sections of accurate and uniform weight, matching and doubling a plurality of the strip sections and hot rolling the doubled sections into sheets or plates of the desired length and gage.

4. The method of making sheets and plates, which consists in cutting long metal slabs of known width and thickness into slabs of the length and weight necessary to make a predetermined number of packs of sheets or plates, and rolling the slabs into long thin flexible strips of known width and gage, then cutting the rolled strips into a predetermined

number of sections and varying the length of the sections into which individual strips are cut to compensate for variations in the temperature at which a series of strips are successively rolled and thereby form duplicate strip sections of accurate and uniform weight, matching and doubling a plurality of the strip sections and hot rolling the doubled sections into sheets or plates of the desired length and gage.

70

5. The method of making sheets and plates, which consists in rolling slabs into long thin flexible strips of known width and gage, then cutting each rolled strip into a predetermined equal number of sections and varying the length of the sections into which individual strips are cut, to compensate for variations in the temperature at which a series of strips are successively rolled and form strip sections of accurate uniform weight matching a plurality of duplicate strip sections and rolling the matched sections into sheets or plates of the desired length and gage.

80

6. The method of making sheets and plates, which consists in rolling slabs of predetermined size and weight into long thin flexible strips of known width and gage, then cutting each rolled strip into a predetermined equal number of sections and varying the length of the sections into which individual strips are cut, to compensate for variations in the temperature at which a series of strips are successively rolled and form strip sections of accurate, uniform weight matching a plurality of duplicate strip sections and rolling the matched sections into sheets or plates of the desired length and gage.

90

7. The method of making sheets and plates, which consists in cutting long metal slabs of known width and thickness into slabs of the length and weight necessary to make a predetermined number of packs of sheets or plates, and rolling the slabs into long thin flexible strips of known width and gage, then cutting each rolled strip into a predetermined number of sections and thereby form strip sections of accurate, uniform weight, then matching and doubling pairs of duplicate strip sections and finally hot rolling the doubled sections to length and gage.

95

8. The method of making sheets and plates, which consists in cutting long metal slabs of known width and thickness into slabs of the length and weight necessary to make a predetermined number of packs of sheets or plates, and rolling the slabs into long thin flexible strips of known width and gage, then cutting each rolled strip into a predetermined number of sections and varying the length of the sections into which the individual strips are cut to compensate for variations in the temperature at which a series of strips are successively rolled and thereby form strip sections of accurate and uniform weight then matching and doubling

100

110

115

120

125

130

pairs of duplicate strip sections, and finally hot rolling the doubled sections to length and gage.

9. The method of making sheets and plates, which consists in cutting long metal slabs of known width and thickness into slabs of the width and weight necessary to make a predetermined number of packs of sheets or plates, and rolling the slabs into long thin

10. flexible strips of known width and gage, then cutting each rolled strip into a predetermined number of sections and varying the length of the sections into which individual strips are cut to compensate for variations

11. in the temperature at which a series of strips are successively rolled and form strip sections of accurate, uniform weight, then matching and doubling pairs of duplicate strip sections, hot rolling the doubled pairs, again doubling the rolled pairs and rolling the twice doubled pairs to length and gage.

10. The method of making sheets and plates, which consists in cutting long metal slabs of known width and thickness into slabs

25. of the width and weight necessary to make a predetermined number of packs of sheets or plates, and rolling the slabs into long thin flexible strips of known width and of from 16 to 18 gage, then cutting each rolled strip

30. into a predetermined number of sections and varying the length of the sections into which individual strips are cut, to compensate for variations in the temperature at which a series of strips are successively rolled and form strip sections of accurate, uniform weight, matching a plurality of duplicate strip sections and hot rolling the matched sections into sheets or plates of the desired length and gage.

40. 11. The method of making sheets and plates, which consists in cutting long metal slabs of known width and thickness into slabs of the length and weight necessary to make a predetermined number of packs of

45. sheets or plates, and rolling the slabs into long thin flexible strips of known width and of from 16 to 18 gage, then cutting each rolled strip into a predetermined number of sections of a length dependent upon the tem-

50. perature at which the slab is rolled and thereby forming strip sections of accurate and uniform weight, matching duplicate strip sections and hot rolling the matched sections into sheets or plates of the desired length and gage.

55. 12. The method of making sheets and plates, which consists in cutting long metal slabs of known width and thickness into slabs of the length and weight necessary to

60. make a predetermined number of packs of sheets or plates, and rolling the slabs into long thin flexible strips of known width and of from 16 to 18 gage, then cutting each rolled strip into a predetermined number of sections and varying the length of the sec-

tions into which individual strips are cut, to compensate for variations in the temperature at which a series of strips are successively rolled and form strip sections of accurate, uniform weight, matching and doubling a plurality of duplicate strip sections and hot rolling the doubled sections into sheets or plates of the desired length and gage.

13. The method of making sheets and plates, which consists in cutting long metal slabs of known width and thickness into slabs of the width and weight necessary to make a predetermined number of packs of sheets or plates, and rolling the slabs into long thin flexible strips of known width and gage, then cutting each rolled strip into a predetermined number of sections and varying the length of the sections into which the individual strips are cut, to compensate for variations in the temperature at which a series of strips are successively rolled and form strip sections of accurate, uniform weight, then matching and doubling a plurality of duplicate strip sections and hot rolling the doubled sections to length and gage.

14. The method of making sheets and plates, which consists in cutting long metal slabs of known width and thickness into slabs of the width and weight necessary to make a predetermined number of packs of sheets or plates, and rolling the slabs into long thin flexible strips of known width and gage, then cutting each rolled strip into a predetermined number of sections and varying the length of the sections into which individual strips are cut, to compensate for variations in the temperature at which a series of strips are successively rolled and form strip sections of accurate, uniform weight, then matching and doubling a plurality of duplicate strip sections and hot rolling the doubled sections to length and gage.

15. The method of making rolled sheets and plates, which consists in rolling slabs into long, thin, flexible strips of known gage and width, stacking the strips as rolled and while still heated from the rolling operation in piles, cooling the piles of strips, then shearing the strips into sections of accurate and uniform weight, matching and doubling a plurality of duplicate strip sections and then heating and rolling the doubled sections to length and gage.

16. The method of making sheets and plates, which consists in cutting long metal slabs of known width and thickness into slabs of the width and gage necessary to make a predetermined number of packs of sheets or plates, and rolling the slabs into long thin flexible strips of known width and gage, then cutting each rolled strip into a predetermined number of sections and varying the length of the sections into which individual strips

re cut, to compensate for variations in the temperature at which a series of strips are successively rolled and form strip sections of accurate, uniform weight, then matching and doubling a plurality of duplicate strip sections, hot rolling the doubled strip sections, again doubling the rolled strip sections and then rolling the twice doubled sections to length and gage.

17. The method of making rolled sheets and plates, which consists in rolling slabs into long, thin, flexible strips of known weight, stacking the strips as rolled and while still heated from the rolling operation in piles, cooling the piles of strips, then shearing each strip into sections of accurate and uniform weight, and then matching and doubling a plurality of duplicate strip sections and heating and rolling the doubled sections to length and gage.

In testimony whereof, I have hereunto signed my name.

CHARLES W. BENNETT.